



US007401912B2

(12) **United States Patent**  
**Pan et al.**

(10) **Patent No.:** **US 7,401,912 B2**  
(45) **Date of Patent:** **Jul. 22, 2008**

(54) **PHASE CHANGE INK IMAGING  
COMPONENT WITH THERMOSET LAYER**

(75) Inventors: **David H. Pan**, Rochester, NY (US);  
**Santokh S. Badesha**, Pittsford, NY (US); **Anthony Yeznach**, Clackamas, OR (US); **Trevor J. Snyder**, Newberg, OR (US); **Barry D. Reeves**, Lake Oswego, OR (US)

(73) Assignee: **Xerox Corporation**, Norwalk, CT (US)

(\*) Notice: Subject to any disclaimer, the term of this patent is extended or adjusted under 35 U.S.C. 154(b) by 232 days.

(21) Appl. No.: **10/922,609**

(22) Filed: **Aug. 19, 2004**

(65) **Prior Publication Data**

US 2006/0038869 A1 Feb. 23, 2006

**Related U.S. Application Data**

(62) Division of application No. 10/177,907, filed on Jun. 20, 2002, now abandoned.

(51) **Int. Cl.**  
**B41J 2/01** (2006.01)

(52) **U.S. Cl.** ..... **347/103; 347/88; 347/99**

(58) **Field of Classification Search** ..... 347/103,  
347/101, 100, 105, 99, 88, 102  
See application file for complete search history.

(56) **References Cited**

**U.S. PATENT DOCUMENTS**

|              |   |         |                     |       |         |
|--------------|---|---------|---------------------|-------|---------|
| 5,372,852 A  | * | 12/1994 | Titterington et al. | ..... | 347/103 |
| 5,536,352 A  | * | 7/1996  | Zeman et al.        | ..... | 156/242 |
| 5,769,957 A  | * | 6/1998  | Murakami et al.     | ..... | 134/15  |
| 6,009,298 A  | * | 12/1999 | Sakamaki et al.     | ..... | 399/318 |
| 6,527,386 B1 | * | 3/2003  | Blank et al.        | ..... | 347/103 |
| 6,648,467 B1 |   | 11/2003 | Pan et al.          |       |         |
| 6,843,559 B2 |   | 1/2005  | Pan et al.          |       |         |
| 6,910,765 B2 |   | 6/2005  | Pan et al.          |       |         |
| 6,918,664 B2 |   | 7/2005  | Pan et al.          |       |         |
| 6,932,470 B2 |   | 8/2005  | Pan et al.          |       |         |
| 6,939,000 B2 |   | 9/2005  | Pan et al.          |       |         |
| 7,234,806 B2 |   | 6/2007  | Pan et al.          |       |         |

\* cited by examiner

*Primary Examiner*—Manish S Shah

(74) *Attorney, Agent, or Firm*—Annette L. Bade

(57) **ABSTRACT**

An offset printing apparatus having a coated imaging drum for use with phase-change inks, wherein the imaging drum including a metal substrate, a conformable intermediate layer, and outer coating having an alkyd thermoset, and a heating member associated with the offset printing apparatus.

**9 Claims, 2 Drawing Sheets**



**FIG. 1****FIG. 2**



**FIG. 3**

**PHASE CHANGE INK IMAGING  
COMPONENT WITH THERMOSET LAYER**

**CROSS-REFERENCE TO RELATED  
APPLICATIONS**

This is a divisional of U.S. application Ser. No. 10/177,907, filed Jun. 20, 2002, now abandoned, by the same inventors, and claims priority therefrom. This divisional application is being filed in response to a restriction requirement in that prior application and contains re-written and/or additional claims to the restricted subject matter.

Reference is made to the following commonly assigned, copending patent applications, including U.S. patent application Ser. No. 10/177,911, filed Jun. 20, 2002, entitled, "Phase Change Ink Imaging Component Having Elastomer Outer Layer;" U.S. patent application Ser. No. 10/177,909, now issued U.S. Pat. No. 6,910,765, U.S. patent application Ser. No. 10/177,780, filed Jun. 20, 2002, entitled, "Phase Change Ink Imaging Component with Thermoplastic Layer;" U.S. patent application Ser. No. 10/177,800, now issued U.S. Pat. No. 7,234,806, U.S. patent application Ser. No. 10/177,906, now issued U.S. Pat. No. 6,918,664, U.S. patent application Ser. No. 10/177,904, now issued U.S. Pat. No. 6,843,559, U.S. patent application Ser. No. 10/177,910, now issued U.S. Pat. No. 6,932,470, U.S. patent application Ser. No. 10/177,779, now issued U.S. Pat. No. 6,648,467, and U.S. patent application Ser. No. 10/177,908, now issued U.S. Pat. No. 6,939,000. The disclosure of each of these patent applications is hereby incorporated by reference in their entirety.

**BACKGROUND**

The present invention relates generally to an imaging apparatus and layers for components thereof, and for use in offset printing or ink jet printing apparatuses. The layers herein are useful for many purposes including layers for transfer components, including transfix or transfuse components, imaging components, and like components. More specifically, the present invention relates to layers comprising a thermoset material. The layers of the present invention may be useful in components used in combination with ink or dye materials. In embodiments, the layers can be used in combination with phase change inks such as solid inks.

Ink jet printing systems using intermediate transfer, transfix or transfuse members are well known, such as that described in U.S. Pat. No. 4,538,156. Generally, the printing or imaging member is employed in combination with a printhead. A final receiving surface or print medium is brought into contact with the imaging surface after the image has been placed thereon by the nozzles of the printhead. The image is then transferred and fixed to a final receiving surface.

More specifically, the phase-change ink imaging process begins by first applying a thin liquid, such as, for example, silicone oil, to an imaging member surface. The solid or hot melt ink is placed into a heated reservoir where it is maintained in a liquid state. This highly engineered ink is formulated to meet a number of constraints, including low viscosity at jetting temperatures, specific visco-elastic properties at component-to-media transfer temperatures, and high durability at room temperatures. Once within the printhead, the liquid ink flows through manifolds to be ejected from microscopic orifices through use of proprietary piezoelectric transducer (PZT) printhead technology. The duration and amplitude of the electrical pulse applied to the PZT is very accurately controlled so that a repeatable and precise pressure pulse can be applied to the ink, resulting in the proper volume,

velocity and trajectory of the droplet. Several rows of jets, for example four rows, can be used, each one with a different color. The individual droplets of ink are jetted onto the liquid layer on the imaging member. The imaging member and liquid layer are held at a specified temperature such that the ink hardens to a ductile visco-elastic state.

After depositing the image, a print medium is heated by feeding it through a preheater and into a nip formed between the imaging member and a pressure member, either or both of which can also be heated. A high durometer synthetic pressure member is placed against the imaging member in order to develop a high-pressure nip. As the imaging member rotates, the heated print medium is pulled through the nip and is pressed against the deposited ink image with the help of a pressure member, thereby transferring the ink to the print medium. The pressure member compresses the print medium and ink together, spreads the ink droplets, and fuses the ink droplets to the print medium. Heat from the preheated print medium heats the ink in the nip, making the ink sufficiently soft and tacky to adhere to the print medium. When the print medium leaves the nip, stripper fingers or other like members, peel it from the printer member and direct it into a media exit path.

To optimize image resolution, the transferred ink drops should spread out to cover a predetermined area, but not so much that image resolution is compromised or lost. The ink drops should not melt during the transfer process. To optimize printed image durability, the ink drops should be pressed into the paper with sufficient pressure to prevent their inadvertent removal by abrasion. Finally, image transfer conditions should be such that nearly all the ink drops are transferred from the imaging member to the print medium. Therefore, it is desirable that the imaging member has the ability to transfer the image to the media sufficiently.

The imaging member is multi-functional. First, the ink jet printhead prints images on the imaging member, and thus, it is an imaging member. Second, after the images are printed on the imaging member, they can then be transfixed or transfused to a final print medium. Therefore, the imaging member provides a transfix or transfuse function, in addition to an imaging function.

In order to ensure proper transfer and fusing of the ink off the imaging member to the print medium, certain nip temperature, pressure and compliance are required. Unlike laser printer imaging technology in which solid fills are produced by sheets of toner, the solid ink is placed on the imaging member one pixel at a time and the individual pixels must be spread out during the transfix process to achieve a uniform solid fill. Also, the secondary color pixels on the imaging member are physically taller than the primary color pixels because the secondary pixels are produced from two primary pixels. Therefore, compliance in the nip is required to conform around the secondary pixels and to allow the primary pixel neighbors to touch the media with enough pressure to spread and transfer. The correct amount of temperature, pressure and compliance is required to produce acceptable image quality.

Currently, the imaging member useful for solid inks or phase change inks comprises anodized aluminum. This member operates at about 57° C. to about 64° C. and can be used with a heater that preheats the print media prior to entering the nip. Otherwise, the imaging member may include a heater associated therewith. The heater may be associated anywhere on the offset printing apparatus. The current aluminum-imaging member has several drawbacks. A high nip load of up to about 770 pounds is needed for transfix or transfuse operations. Further, because of the high nip load, bulky mechan-

nisms and supporting structures are needed, resulting in increased printer weight and cost. One example is that a fairly complex two-layer pressure roller is needed. In addition, the first copy out time is unacceptable because of the bulky weight. Moreover, low cohesive failure temperature is another drawback to use of an anodized aluminum drum.

Several coatings for the imaging member have been suggested. Examples are listed below.

U.S. Pat. No. 5,092,235 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60.

U.S. Pat. No. 5,195,430 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60, which can be polyurethane (VIBRATHANE, or REN:C: O-thane).

U.S. Pat. No. 5,389,958 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), and a pressure roller with elastomer surface.

U.S. Pat. No. 5,455,604 discloses a fixing mechanism and pressure wheels, wherein the pressure wheels can be comprised of a steel or plastic material such as DELRIN. Image-receiving drum **40** can be a rigid material such as aluminum or stainless steel with a thin shell mounted to the shaft, or plastic.

U.S. Pat. No. 5,502,476 teaches a pressure roller having a metallic core with elastomer coating such as silicones, urethanes, nitriles, or EPDM, and an intermediate transfer member surface of liquid, which can be water, fluorinated oils, glycol, surfactants, mineral oil, silicone oil, functional oils such as mercapto silicone oils or fluorinated silicone oils or the like, or combinations thereof.

U.S. Pat. No. 5,614,933 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,790,160 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,805,191 an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and an outer liquid layer of liquid, which can be water, fluorinated oils, glycol, surfactants, mineral oil, silicone oil, functional oils such as mercapto silicone oils or fluorinated silicone oils or the like, or combinations thereof.

U.S. Pat. No. 5,808,645 discloses a transfer roller having a metallic core with elastomer covering of silicone, urethanes, nitriles, and EPDM.

U.S. Pat. No. 6,196,675 B1 discloses separate image transfer and fusing stations, wherein the fuser roller coatings can be silicones, urethanes, nitrates and EPDM.

U.S. Pat. No. 5,777,650 discloses a pressure roller having an elastomer sleeve, and an outer coating that can be metals, (aluminum, nickel, iron phosphate), elastomers (fluoroelastomers, perfluoroelastomers, silicone rubber, polybutadiene), plastics (polyphenylene sulfide with PTFE filler), thermoplastics (polyethylene, polyamide (nylon), FEP), thermosets (acetals, ceramics). Preferred is anodized aluminum.

In addition, many different types of outer coatings for transfer members, fuser members, and intermediate transfer members have been used in the electrostatographic arts using powder toner, but not with liquid inks or phase change inks. Several examples are listed herein.

U.S. Pat. No. 5,361,126 discloses an imaging apparatus including a transfer member including a heater and pressure-applying roller, wherein the transfer member includes a fabric substrate and an impurity-absorbent material as a top layer. The impurity-absorbing material can include a rubber elastomer material.

U.S. Pat. No. 5,337,129 discloses an intermediate transfer component comprising a substrate and a ceramer or grafted ceramer coating comprised of integral, interpenetrating networks of haloelastomer, silicon oxide, and optionally polyorganosiloxane.

U.S. Pat. No. 5,340,679 discloses an intermediate transfer component comprised of a substrate and thereover a coating comprised of a volume grafted elastomer, which is a substantially uniform integral interpenetrating network of a hybrid composition of a fluoroelastomer and a polyorganosiloxane.

U.S. Pat. No. 5,480,938 describes a low surface energy material comprising a volume grafted elastomer which is a substantially uniform integral interpenetrating network of a hybrid composition of a fluoroelastomer and a polyorganosiloxane, the volume graft having been formed by dehydrofluorination of fluoroelastomer by a nucleophilic dehydrofluorinating agent, followed by a hydrosilation reaction, addition of a hydrogen functionally terminated polyorganosiloxane and a hydrosilation reaction catalyst.

U.S. Pat. No. 5,366,772 describes a fuser member comprising a supporting substrate, and a outer layer comprised of an integral interpenetrating hybrid polymeric network comprised of a haloelastomer, a coupling agent, a functional polyorganosiloxane and a crosslinking agent.

U.S. Pat. No. 5,456,987 discloses an intermediate transfer component comprising a substrate and a titamer or grafted titamer coating comprised of integral, interpenetrating networks of haloelastomer, titanium dioxide, and optionally polyorganosiloxane.

U.S. Pat. No. 5,848,327 discloses an electrode member positioned near the donor member used in hybrid scavengerless development, wherein the electrode members have a composite haloelastomer coating.

U.S. Pat. No. 5,576,818 discloses an intermediate toner transfer component including: (a) an electrically conductive substrate; (b) a conformable and electrically resistive layer comprised of a first polymeric material; and (c) a toner release layer comprised of a second polymeric material selected from the group consisting of a fluorosilicone and a substantially uniform integral interpenetrating network of a hybrid composition of a fluoroelastomer and a polyorganosiloxane, wherein the resistive layer is disposed between the substrate and the release layer.

U.S. Pat. No. 6,035,780 discloses a process for forming a layer on a component of an electrostatographic apparatus, including mixing a first fluoroelastomer and a polymeric siloxane containing free radical reactive functional groups, and forming a second mixture of the resulting product with a mixture of a second fluoroelastomer and a second polysiloxane compound.

U.S. Pat. No. 5,537,194 discloses an intermediate toner transfer member comprising: (a) a substrate; and (b) an outer layer comprised of a haloelastomer having pendant hydrocarbon chains covalently bonded to the backbone of the haloelastomer.

U.S. Pat. No. 5,753,307 discloses fluoroelastomer surfaces and a method for providing a fluoroelastomer surface on a supporting substrate which includes dissolving a fluoroelastomer; adding a dehydrofluorinating agent; adding an amino silane to form a resulting homogeneous fluoroelastomer solution; and subsequently providing at least one layer of the homogeneous fluoroelastomer solution to the supporting substrate.

U.S. Pat. No. 5,840,796 describes polymer nanocomposites including a mica-type layered silicate and a fluoroelastomer, wherein the nanocomposite has a structure selected from the group consisting of an exfoliated structure and an intercalated structure.

U.S. Pat. No. 5,846,643 describes a fuser member for use in an electrostatographic printing machine, wherein the fuser member has at least one layer of an elastomer composition comprising a silicone elastomer and a mica-type layered silicate, the silicone elastomer and mica-type layered silicate form a delaminated nanocomposite with silicone elastomer inserted among the delaminated layers of the mica-type layered silicate.

It is desired to provide a multi-functional imaging member for use with phase change ink printing machines, which has the ability to receive an image, and either transfer or transfer and fuse the image to a print medium. It is desired that the imaging member when having heat associated therewith, be thermally stable for conduction for fusing or fixing. It is further desired that the imaging member have a relatively low nip load, in order to decrease the weight and cost of the printing machine, and in order to provide an acceptable first copy out time.

## SUMMARY

The present invention provides, in embodiments: an offset printing apparatus for transferring a phase change ink onto a print medium comprising: a) a phase change ink component for applying a phase change ink in a phase change ink image; b) an imaging member for accepting the phase change ink image from the phase change ink component, and transferring the phase change ink image from the imaging member to the print medium, the imaging member comprising: i) an imaging substrate, and thereover ii) an outer coating comprising a thermoset other than ceramics and silicones.

The present invention further provides, in embodiments: an offset printing apparatus for printing a phase change ink onto a print medium comprising: a) a phase change ink component for applying a phase change ink in a phase change ink image; b) an imaging member for accepting said phase change ink image from said phase change ink component, and transferring the phase change ink image from said imaging member to said print medium and for fixing the phase change ink image to said print medium, the imaging member comprising in order: i) an imaging substrate, ii) an intermediate layer, and

iii) an outer coating comprising a thermoset other than ceramics and silicones; and c) a heating member associated with the offset printing apparatus.

In addition, the present invention provides, in embodiments: an offset printing apparatus comprising a phase change ink component containing a phase change ink; an imaging member comprising a substrate, and thereover an outer coating comprising a thermoset other than ceramics and silicones, and a heating member associated with the offset printing apparatus, wherein the phase change ink component dispenses the phase change ink onto the imaging member, and wherein the phase change ink is solid at room temperature.

## BRIEF DESCRIPTION OF THE DRAWINGS

The above embodiments of the present invention will become apparent as the following description proceeds upon reference to the drawings, which include the following figures:

FIG. 1 is an illustration of an embodiment of the invention, and includes a transfer printing apparatus using an imaging member in the form of a drum.

FIG. 2 is an enlarged view of an embodiment of a printing drum having a substrate and an outer elastomer layer thereon.

FIG. 3 is an enlarged view of an embodiment of a printing drum having a substrate, an optional intermediate layer, and an outer thermoset layer thereon.

## DETAILED DESCRIPTION

The present invention is directed to an offset printing apparatus useful with phase-change inks such as solid inks, and comprising a coated imaging member capable of accepting, transferring and in some embodiments, fixing an ink image to a print medium. The imaging member can be a roller such as a drum, or a film component such as a film, sheet, belt or the like. In embodiments, the imaging member comprises a substrate and an outer layer comprising a thermoset. In an alternative embodiment, the imaging member comprises a substrate, an optional intermediate layer, and outer layer comprising a thermoset. The substrate, intermediate layer, and/or outer layer can further comprise fillers dispersed or contained therein.

The details of embodiments of phase-change ink printing processes are described in the patents referred to above, such as U.S. Pat. Nos. 5,502,476; 5,389,958; and 6,196,675 B1, the disclosures of each of which are hereby incorporated by reference in their entirety.

Referring to FIG. 1, offset printing apparatus 1 is demonstrated to show transfer of an ink image from the imaging member to a final printing medium or receiving substrate. As the imaging member 3 turns in the direction of arrow 5, a liquid surface 2 is deposited on imaging member 3. The imaging member 3 is depicted in this embodiment as a drum member. However, it should be understood that other embodiments can be used, such as a belt member, film member, sheet member, or the like. The liquid layer 2 is deposited by an applicator 4 that may be positioned at any place, as long as the applicator 4 has the ability to make contact and apply liquid surface 2 to imaging member 3.

The ink used in the printing process can be a phase change ink, such as, for example, a solid ink. The term "phase change ink" means that the ink can change phases, such as a solid ink becoming liquid ink or changing from solid into a more malleable state. Specifically, in embodiments, the ink can be in solid form initially, and then can be changed to a molten state by the application of heat energy. The solid ink may be

solid at room temperature, or at about 25° C. The solid ink may possess the ability to melt at relatively high temperatures above from about 85° C. to about 150° C. The ink is melted at a high temperature and then the melted ink **6** is ejected from printhead **7** onto the liquid layer **2** of imaging member **3**. The ink is then cooled to an intermediate temperature of from about 20° C. to about 80° C., or about 72° C., and solidifies into a malleable state in which it can then be transferred onto a final receiving substrate **8** or print medium **8**.

The ink has a viscosity of from about 5 to about 30 centipoise, or from about 8 to about 20 centipoise, or from about 10 to about 15 centipoise at about 140° C. The surface tension of suitable inks is from about 23 to about 50 dynes/cm. Examples of a suitable inks for use herein include those described in U.S. Pat. Nos. 4,889,560; 5,919,839; 6,174,937; and 6,309,453, the disclosure each of which are hereby incorporated by reference in their entirety.

Some of the liquid layer **2** is transferred to the print medium **8** along with the ink. A typical thickness of transferred liquid is about 100 angstroms to about 100 nanometer, or from about 0.1 to about 200 milligrams, or from about 0.5 to about 50 milligrams, or from about 1 to about 10 milligrams per print medium.

Suitable liquids that may be used as the print liquid surface **2** include water, fluorinated oils, glycol, surfactants, mineral oil, silicone oil, functional oils, and the like, and mixtures thereof. Functional liquids include silicone oils or polydimethylsiloxane oils having mercapto, fluoro, hydride, hydroxy, and the like functionality.

Feed guide(s) **10** and **13** help to feed the print medium **8**, such as paper, transparency or the like, into the nip **9** formed between the pressure member **11** (shown as a roller), and imaging member **3**. It should be understood that the pressure member can be in the form of a belt, film, sheet, or other form. In embodiments, the print medium **8** is heated prior to entering the nip **9** by heated feed guide **13**. When the print medium **8** is passed between the printing medium **3** and the pressure member **11**, the melted ink **6** now in a malleable state is transferred from the imaging member **3** onto the print medium **8** in image configuration. The final ink image **12** is spread, flattened, adhered, and fused or fixed to the final print medium **8** as the print medium moves between nip **9**. Alternatively, there may be an additional or alternative heater or heaters (not shown) positioned in association with offset printing apparatus **1**. In another embodiment, there may be a separate optional fusing station located upstream or downstream of the feed guides.

The pressure exerted at the nip **9** is from about 10 to about 1,000 psi, or about 500 psi, or from about 200 to about 500 psi. This is approximately twice the ink yield strength of about 250 psi at 50° C. In embodiments, higher temperatures, such as from about 72 to about 75° C. can be used, and at the higher temperatures, the ink is softer. Once the ink is transferred to the final print medium **8**, it is cooled to an ambient temperature of from about 20° C. to about 25° C.

Stripper fingers (not shown) may be used to assist in removing the print medium **8** having the ink image **12** formed thereon to a final receiving tray (also not shown).

FIG. 2 demonstrates an embodiment of the invention, wherein imaging member **3** comprises substrate **15**, having thereover outer coating **16**.

FIG. 3 depicts another embodiment of the invention. FIG. 3 depicts a three-layer configuration comprising a substrate **15**, intermediate layer **17** positioned on the substrate **15**, and outer layer **16** positioned on the intermediate layer **17**. In embodiments, an outer liquid layer **2** (as described above) may be present on the outer layer **16**.

In embodiments, the outer release layer **16** comprises a thermoset. In embodiments, the thermoset is a thermoset other than ceramics and silicones.

A thermoset material is a polymer that solidifies or "sets" irreversibly when heated. Usually, the polymer is covalently cross-linked using radiation or the like, in order to provide the thermoset or thermally stable elastomeric property. In some cases, curing agents or other additives may be added in order to provide the thermoset property.

In general, cross-linked thermoset network materials have excellent dimensional stability under heat, pressure or even solvent exposure, and are tough, have easy to tailor hardness, and are chemically inert. Their surface energy can be tailored by incorporating low surface energy segments into the network, such as in the example of siloxane urethane family of thermoset materials. The thermoset materials exhibit substantial advantages over ceramics and silicones disclosed as being used in the art. One of the typical advantages is that it is extremely difficult to make ceramics in the Shore D or pencil hardness range, and on the contrary, unfilled silicones are just too soft to achieve much higher hardness using several known approaches.

A lot of thermoplastics can be made into their thermoset equivalents. By definition, thermoplastic polymers are usually linear or branched polymers and do not form a network having infinite molecular weight. Thus dimensions of thermoplastic polymers can be formed and changed by heat, pressure or solvent and reversibly reformed into the same. Linear polymers are polymerized from substantially bi-functional monomers. However, if some bi-functional monomers are replaced by monomers having functionality greater or equal to 3, a network or thermoset polymer is thus formed. A typical example is linear or thermoplastic polystyrene from styrene or fluorinated styrene monomers, but if some divinylbenzene—a tetrafunctional monomer is added to styrene or fluorinated styrene monomers, a cross-linked or thermoset polystyrene can be formed. The thermoset once formed will not flow or reversibly re-shape or be reused. In fact, another well-known example is that there are thermoplastic and thermoset polyurethanes. The difference between the two could be simply di-isocyanate versus tri or tetra-isocyanate monomers and, alternatively, di-ol versus tri-ol or tetra-ol monomers or soft segments. Similarly, linear polymers, given the right chemistry, can be made into thermoset polymers by using high-energy radiation, such as  $\gamma$ -ray.

Examples of suitable thermosets include urethanes such as polyurethanes, polysiloxane-based urethanes, fluoropolymer-based urethanes, polyester-based urethanes, polyether-based urethanes and polycaprolactone-based urethanes, available from Uniroyal, Bayer, Conap, and the like.

Other examples of thermosets include phenolics. In addition, examples of thermosets include amino resins (such as condensation products of urea and melamine with formaldehyde); unsaturated polyester resins; air-drying oils based on unsaturated fatty acids which cure by oxidation of the acids; alkyds which are cross-linked polyesters primarily based on phthalic anhydride and glycerol or other polyhydric alcohols (many alkyd resins are modified by the addition of unsaturated fatty acids such as drying oils); epoxies, and the like, and mixtures thereof. Other examples include natural (isoprene) rubbers and chlorinated rubbers, polysulfide rubbers, rubbers derived from butadiene such as styrene butadiene rubbers, chloroprene (neoprene) rubbers, ethylene propene diene elastomers such as ion-containing ethylene propene diene elastomers, nitrile rubbers, and sol-gel resins (condensation products of metal alkoxides and organic polymers, such as polysilazane rubbers, polyphosphazene rubbers, and pol-

polysilsesquioxane resins such as TRIPLUS® 178 or TRIPLUS® 179 from GE Silicones, also known as T-resins R—SiO<sub>1.5</sub> or Q-resins). Polysilsesquioxane or functionalized polysilsesquioxane resins can be co-polymerized with a variety of monomers to form hybrid organic-inorganic thermoset materials, hetrosilsesquioxane and metallasilsesquioxane resins. Mixtures of thermosets can also be used.

In embodiments, the thickness of the outer thermoset imaging layer is from about 0.5 to about 20 mils, or from about 0.5 to about 6 mils.

The substrate, optional intermediate layer, and/or outer layer, in embodiments, may comprise fillers dispersed therein. These fillers can have the ability to increase the material hardness or modulus into the desired range.

Examples of fillers include fillers such as metals, metal oxides, doped metal oxides, carbon blacks, ceramics, silicates (such as zirconium silicate, mica and the like), polymers, and the like, and mixtures thereof. Examples of suitable metal oxide fillers include titanium dioxide, tin (II) oxide, aluminum oxide, indium-tin oxide, magnesium oxide, copper oxide, iron oxide, silica or silicon oxide, and the like, and mixtures thereof. Examples of carbon fillers include carbon black (such as N-990 thermal black, N330 and N110 carbon blacks, and the like), graphite, fluorinated carbon (such as ACCUFLUOR® or CARBOFLUOR®), and the like, and mixtures thereof. Examples of ceramic materials include aluminum nitrate, boron nitride, silicates such as zirconium silicates, and the like, and mixtures thereof. Examples of polymer fillers include polytetrafluoroethylene powder, polypyrrole, polyacrylonitrile (for example, pyrolyzed polyacrylonitrile), polyaniline, polythiophenes, and the like, and mixtures thereof. The optional filler is present in the substrate, optional intermediate layer, and/or outer layer in an amount of from about 0 to about 60 percent, or from about 1 to about 20 percent, or from about 1 to about 5 percent by weight of total solids in the layer.

The imaging substrate can comprise any material having suitable strength for use as an imaging member substrate. Examples of suitable materials for the substrate include metals, fiberglass composites, rubbers, and fabrics. Examples of metals include steel, aluminum, nickel, and their alloys, and like metals, and alloys of like metals. The thickness of the substrate can be set appropriate to the type of imaging member employed. In embodiments wherein the substrate is a belt, film, sheet or the like, the thickness can be from about 0.5 to about 500 mils, or from about 1 to about 250 mils. In embodiments wherein the substrate is in the form of a drum, the thickness can be from about 1/32 to about 1 inch, or from about 1/16 to about 5/8 inch.

Examples of suitable imaging substrates include a sheet, a film, a web, a foil, a strip, a coil, a cylinder, a drum, an endless strip, a circular disc, a belt including an endless belt, an endless seamed flexible belt, an endless seamless flexible belt, an endless belt having a puzzle cut seam, a weldable seam, and the like.

In an optional embodiment, an intermediate layer may be positioned between the imaging substrate and the outer layer. Materials suitable for use in the intermediate layer include silicone materials, fluoroelastomers, fluorosilicones, ethylene propylene diene rubbers, and the like, and mixtures thereof. In embodiments, the intermediate layer is conformable and is of a thickness of from about 2 to about 60 mils, or from about 4 to about 25 mils.

Specific embodiments of the invention will now be described in detail. These examples are intended to be illustrative, and the invention is not limited to the materials, conditions, or process parameters set forth in these embodiments.

All parts are percentages by weight of total solids as defined above unless otherwise indicated.

## EXAMPLES

### Example 1

#### Preparation of a Thermoset Outer Imaging Layer

Polysilsesquioxane resin layer containing GE TRIPLUS®

178, TRIPLUS® 179 and carbon black filler can be prepared according to the following formulation:

TABLE I

| Material                            | Parts by weight |
|-------------------------------------|-----------------|
| TriPlus 178                         | 50              |
| TriPlus 179                         | 50              |
| N330 Carbon Black                   | 20              |
| Zirconium 2-ethylhexanoate catalyst | 0.25            |

An amount of about 20 grams of N330 carbon black can be first dispersed in the mixture of 50 grams of TRIPLUS® 178 and 50 grams of TRIPLUS® 179 by using an appropriate paint-shaker filled with some 3/8" ceramic shots for about 16 hours. The dispersion can then be combined and homogenized with 0.25 grams of zirconium 2-ethylhexanoate catalyst and dispersed by paint-shaking for about 15 minutes. A prototype polysilsesquioxane layer can then be applied by coating the above dispersion onto a stainless steel substrate. The coated layer can be cured in oven at the following conditions: 10 minutes at 70-90° C., 10 minutes at 125-150° C. and 60 minutes at 250° C.

### Example 2

#### Preparation of Imaging Drums

The dispersion made in accordance with Example 1 can be coated onto an aluminum imaging drum of approximately 100 mm in diameter. Prior to coating the aluminum drum is grit blasted and degreased with methyl ethyl ketone solvent and dried. The coating is then applied using known methods such as flow coating, spray coating, dip coating, gravure coating, roll coating, and the like. The resulting drum is then dried and step cured.

While the invention has been described in detail with reference to specific and preferred embodiments, it will be appreciated that various modifications and variations will be apparent to the artisan. All such modifications and embodiments as may readily occur to one skilled in the art are intended to be within the scope of the appended claims.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others.

What is claimed is:

1. An offset printing apparatus for printing a phase change ink onto a print medium comprising:
  - a phase change ink component for applying a phase change ink in a phase change ink image;
  - an imaging drum for accepting said phase change ink image from said phase change ink component, and transferring the phase change ink image from said drum to said print medium and for fixing the phase change ink image to said print medium, the imaging drum comprising in order:

**11**

- i) an imaging drum comprising a metal substrate,
  - ii) a conformable intermediate layer, and
  - iii) an outer coating comprising an alkyd thermoset;
  - c) a pressure member in pressure contact with said imaging drum, wherein said print medium is fed through a nip formed between said imaging member and said pressure member, and wherein a pressure exerted at said nip is from about 200 to about 500 psi; and
  - d) a heating member associated with the offset printing apparatus.
2. The offset printing apparatus of claim 1, wherein said outer coating further comprises a filler.
3. The offset printing apparatus of claim 2, wherein said filler is selected from the group consisting of metals, metal oxides, carbon blacks, polymers, and mixtures thereof.

**12**

- 4. The offset printing apparatus of claim 1, wherein said intermediate layer comprises a silicone material.
- 5. The offset printing apparatus of claim 1, wherein said intermediate layer further comprises a filler.
- 5. The offset printing apparatus of claim 5, wherein said filler is selected from the group consisting of carbon blacks, metal oxides, metals, polymers, and mixtures thereof.
- 7. The offset printing apparatus of claim 1, wherein said phase change ink is solid at about 25° C.
- 8. The offset printing apparatus of claim 1, wherein said phase change ink comprises a dye.
- 9. The offset printing apparatus of claim 1, wherein said conformable intermediate layer has a thickness of from about 2 to about 60 mils.

\* \* \* \* \*